

1

3,364,232

SULFUR CONTAINING PSEUDOAROMATIC  
DETERGENTS

Donald J. Anderson, San Anselmo, Calif., assignor to  
Chevron Research Company, San Francisco, Calif., a  
corporation of Delaware  
No Drawing. Filed Jan. 5, 1966, Ser. No. 518,787  
5 Claims. (Cl. 260—327)

This invention concerns novel pseudo-aromatic sulfur containing compounds and their use as detergents in lubricating oils. More particularly, this invention concerns relatively high molecular weight hydrocarbon substituted pseudo-aromatic compounds having annular sulfur and their use as detergents in lubricating oils.

Trithiones are a peculiar type of pseudo-aromatic system in having only one double bond in a five-membered ring and the inability to introduce a second conventional double bond. Trithione compounds are readily prepared by the reaction of olefins having at least one methyl group and have been reported for a variety of uses. See, for example, U.S. Patent Nos. 2,535,705 and 2,658,900. However, for the most part, the trithiones have been of relatively low molecular weight. The most commonly reported trithiones in the patent literature have been the trithiones of isobutylene and diisobutylene.

It has now been found that trithiones having a molecular weight of at least about 500 and a hydrocarbon alkyl substituent of at least about 30 carbon atoms can be prepared and find use as detergents in lubricating oils. Generally, the trithiones will have molecular weights of less than 5,000 and usually less than 3,000.

For the most part, the trithiones of this invention will have the following formula:



wherein  $R^1$  and  $R^2$  have a total number of carbon atoms in the range of 30 to 325, at least one being aliphatic hydrocarbon and the other being hydrogen or aliphatic hydrocarbon; usually one of  $R^1$  and  $R^2$  is an aliphatic hydrocarbon group of from about 30 to 325 carbon atoms, more usually from about 50 to 125 carbon atoms and the other may be hydrogen or lower alkyl. The total molecular weight is in the range of about 500 to 5,000, more usually about 750 to 3,000.

Generally, the compositions of this invention will come within the following formula:



wherein  $R^3$  is an aliphatic hydrocarbon group of from about 30 to 325 carbon atoms, preferably from about 50 to 175 carbon atoms and particularly preferred from about 50 to 125 carbon atoms, and  $R^4$  is lower alkyl of from 1 to 6 carbon atoms or hydrogen, usually methyl.

The aliphatic hydrocarbon substituents may be derived from a variety of sources, may be branched chain or straight chain, and while they may include cycloaliphatic groups, for the most part they will be acyclic.

Sources of hydrocarbons having the necessary number of carbon atoms include petroleum fractions, polymers of olefins of from about 2 to 6 carbon atoms, more usually from about 2 to 5 carbon atoms, e.g., propylene, isobutene, butenes, 4-methyl-1-pentene, etc.

The preferred aliphatic hydrocarbons are those derived from olefins of from about 3 to 4 carbon atoms, i.e., propylene and isobutylene; that is, polymers which are branched chain. Of course, ethylene may be copoly-

2

erized with olefins of a higher number of carbon atoms to provide branched chain aliphatic hydrocarbon groups.

Illustrative compounds include 5-n-alkyl trithione, 5-polypropylene trithione, 5-polyisobutylene trithione, 5-(copolymer of ethylene and isobutylene prepared by the cationic polymerization of 4-methylpentene-1) trithione, 4-methyl polyisobutylene trithione, etc.

If desired, the trithione may be oxidized with a peroxidic compound to form the S-oxy trithione. This compound is believed to have the following formula:



wherein  $R^1$  and  $R^2$  are as defined previously.

The following formula:



wherein  $R^1$  and  $R^2$  are as defined previously and  $X$  is either a pair of unshared electrons or coordinately bonded oxygen, may be considered generic to the trithione and its oxy derivative.

While the trithiones of low molecular weight are readily prepared by contacting sulfur with an olefin of the following basic structure:



or a compound which fulfills the function of an olefin in the reaction, e.g., an aliphatic ketone, it is found that with the high molecular weight polyolefins, e.g., polyisobutylene, a low molecular weight trithione must be present in order to obtain the trithiones of this invention. That is, the high molecular weight olefin, i.e., of at least 30 carbon atoms, is contacted with sulfur in the presence of approximately equimolar amounts of the high molecular weight olefin and a trithione of from about 4 to 16 carbon atoms, preferably of from about 8 to 12 carbon atoms and from about a 5 to 100 weight percent excess of the stoichiometric amount of sulfur and the mixture heated at temperatures in excess of 175° C. and generally less than 275° C. for periods ranging from about 2 to 24 hours. By distilling off the low molecular weight materials, the desired trithione compound may be directly isolated.

The oxy derivative may then be prepared by dissolving the trithione in a suitable inert solvent, e.g., benzene, and then adding hydrogen peroxide at ambient temperatures in the presence of a hydroxylc organic solvent, e.g., methanol, acetic acid, etc.

The product formed as described above may then be used in a variety of lubricating oils as detergents.

The following examples are offered by way of illustration and not by way of limitation.

Example I

60 Into a reaction flask in a nitrogen atmosphere was introduced 160 g. (5 gram atoms) of sulfur and 260 g. of 4 - neopentyl - 5 - tert-butyl - 1,2 - dithiol-3-thione, the mixture heated at 200° C. in a nitrogen atmosphere, and 900 g. (approximately 1 mole) of polyisobutylene added over a period of about an hour. The temperature was maintained for 12 hours, at the end of which time the temperature was raised to 210° C. and the pressure reduced to about 4-5 mm. Hg and any volatile material distilled overhead. The residue weighed 1,028 g. Analysis: S=10.0, 10.1. An infrared spectrum of the product was consistent with the trithione.

3  
*Example II*

Following the procedure of Example I, 900 g. of polyisobutylene (approximately 1 mole), 160 g. of sulfur (5 gram atoms), and 260 g. of the same low molecular weight trithione (approximately 1 mole) were mixed in a nitrogen atmosphere. At the end of the heating period, the temperature was raised to 250° C. and the pressure reduced to 3 mm. Hg. The residue weighed 766 g. Analysis: S=6.5.

*Example III*

Into a reaction flask was charged 1,500 g. (approximately 1.5 moles) of polyisobutylene trithione (approximately 8 weight percent sulfur) and 1.5 liters of benzene and stirred while 170.3 g. (approximately 1.5 moles) of hydrogen peroxide (30 weight percent aqueous solution) was added over a period of 30 minutes. The mixture was then stirred for an additional 2.5 hours, followed by the addition of 50 ml. of methanol. When it appeared that no reaction had occurred, 10 ml. of acetic acid was added and the temperature increased to 58° C. This seemed to initiate the reaction, the temperature was allowed to drop to 50° C. and the reaction mixture then held at that temperature. When no further reaction appeared to be occurring, the product was washed with water, and the organic phase dried over sodium sulfate, filtered and stripped in vacuo. The residue weighed approximately 1,300 g. Analysis: S=10.0.

*Example IV*

(A) Into a reaction flask was introduced 260 g. (1 mole) of polyisobutylene trithione and 370 g. (10 g. atoms) of sulfur, and the reaction flask flushed with nitrogen. The mixture was then heated to 200° C. and 900 g. (2 moles) of polyisobutylene added over a period of 7 hours. Heating was continued at the same temperature for a further 14 hours. Volatile materials were then removed by heating the mixture to 240° C. with a stream of nitrogen bubbling through the mixture. The product weighed 770 g. Analysis: S=12.7, 12.9; molecular weight (ThermoNAM—Differential Vapor Pressure Technique)=770.

(B) The above procedure was repeated using the same amount of materials. The product weighed 806 g. Analysis: S=13.1, 13.2; molecular weight (ThermoNAM)=691.

As already indicated, the compounds of this invention

excellent compatibility with oils. As concentrates, the compounds of this invention will generally range from about 20 to 80 weight percent of the total composition, more usually from about 40 to 70 weight percent.

5 A preferred aspect in using the compounds of this invention in lubricating oils is to include in the oil from about 1 to 50 mm./kg. of an O,O-dihydrocarbyl phosphorodithioate, particularly a zinc salt, wherein the hydrocarbyl groups are from about 4 to 36 carbon atoms. (Hydrocarbyl is a monovalent organic radical composed solely of carbon and hydrogen which may be aliphatic, alicyclic or aromatic, or combinations thereof, e.g., aralkyl.) Instead of zinc, an alkyl group or polyethyleneoxy group may also be used. Generally, the hydrocarbyl 10 groups will be alkyl or alkaryl.

The lubricating fluids which may be used with the compounds of this invention (hereinafter referred to as oils) may be derived from natural or synthetic sources. Oils generally have viscosities of from about 35 to 50,000 15 Saybolt Universal Seconds (SUS) at 100° F. Among natural hydrocarbonaceous oils are paraffin base, naphthenic base, asphaltic base and mixed base oils. Illustrative synthetic oils are: hydrocarbon oils, such as polymers of various olefins, generally of from 2 to 8 carbon atoms, and alkylated aromatic hydrocarbons; and non-hydrocarbon oils, such as polyalkylene oxides, aromatic ethers, carboxylate esters, phosphate esters and silicon esters. The preferred media are the hydrocarbonaceous 20 media, both natural and synthetic.

25 30 The above oils may be used individually or together, whenever miscible or made so by the use of mutual solvents.

Other additives may also be included in the oils such as pour point depressants, oiliness agents, antioxidants, 35 rust inhibitors, etc. Usually, the total amount of the additives will range from about 0.1 to 10 weight percent, more usually from about 0.5 to 5 weight percent. The individual additives may vary from about 0.01 to 5 weight percent.

40 In order to demonstrate the excellent effectiveness of the compounds of this invention as detergents and dispersants in lubricating oils, the compounds prepared were tested in the 1-G Caterpillar Test (MIL-L-45199 conditions). The oil used was a Mid-Continent SAE 30 oil and 45 12 mm./kg. of zinc di(alkylphenyl) phosphorodithioate (the alkyl groups were polypropylene of about 12 to 15 carbon atoms) was included. The test was carried out for 60 hours and in some instances 120 hours. The following table indicates the results.

TABLE I

| Example         | Wt. percent of detergent in oil composition | 60 Hours                     |                            |                        | 120 Hours       |               |           |
|-----------------|---------------------------------------------|------------------------------|----------------------------|------------------------|-----------------|---------------|-----------|
|                 |                                             | Groove <sup>1</sup> Deposits | Land <sup>2</sup> Deposits | Underhead <sup>3</sup> | Groove Deposits | Land Deposits | Underhead |
| I               | 5                                           | 15- 3-0-0                    | 100- 5-10                  | 7.5                    | 87-7-3-2        | 440-330-390   | 3.8       |
| II              | 10                                          | 21- 5-0-0                    | 95- 0-0                    | 7.5                    | 51-8-0-0        | 465- 55- 30   | 5.6       |
| III             | 5                                           | 46- 5-0-0                    | 145- 0-0                   | 7.5                    | -----           | -----         | -----     |
| IV <sup>4</sup> | 10                                          | 50- 9-0-1                    | 480-240-490                | -----                  | -----           | -----         | -----     |
| Base oil        |                                             | 93-15-5-3                    | 500-300-370                | -----                  | -----           | -----         | -----     |

<sup>1</sup> Groove deposits are rated on a scale of 0 to 100, 0 being completely clean and 100 being completely filled.

<sup>2</sup> Land deposits rated on a scale of 0 to 800, 0 being completely clean and 800 being completely black.

<sup>3</sup> Underhead rated on a scale of 0 to 10, 0 being completely black and 10 being completely clean.

<sup>4</sup> The results were obtained in the absence of any zinc dithiophosphate in the oil.

find use as dispersants and detergents in lubricating oils. They are of particular value in diesel engines, demonstrating excellent results under the high temperatures at which diesel engines operate. When compounded with a lubricating oil for use in an engine, the compounds of this invention will be present in at least about 0.1 weight percent and usually not more than 20 weight percent, more usually in the range of about 2 to 15 weight percent. The detergents of this invention may be used with other detergents or by themselves. The compounds of this invention can be prepared as concentrates due to their

65 It is obvious from the above results that the compositions of this invention are excellent detergents under the extremely severe high temperatures at which diesel engines are operated. Moreover, the detergents are compatible with a common lubricating oil additive, namely the phosphorodithioate.

70 75 As will be evident to those skilled in the art, various modifications on this invention can be made or followed, in the light of the foregoing disclosure and discussion, without departing from the spirit or scope of the disclosure or from the scope of the following claims.

What is claimed is:

1. A composition having a molecular weight in the range of 750 to 3,000 and of the formula:



wherein  $R^1$  and  $R^2$  are alkyl or hydrogen, at least one of  $R^1$  and  $R^2$  being alkyl.

2. A composition according to claim 1, wherein  $R^1$  and  $R^2$  have a total of from 50 to 125 carbon atoms.

3. A composition according to the formula:



wherein  $R^1$  and  $R^2$  are alkyl or hydrogen having a total of from 50 to 175 carbon atoms, at least one of  $R^1$  and  $R^2$  being alkyl.

4. A composition according to claim 3, wherein  $R^1$  and  $R^2$  have from 50 to 125 carbon atoms.

5. A method of preparing a composition according to claim 1, which comprises contacting at a temperature in excess of 175° C. an aliphatic monoolefin of at least 30 carbon atoms having a group of the formula:



with sulfur in from 5 to 100 percent excess of the stoichiometric amount of sulfur required, in the presence of a trithione of from 4 to 16 carbon atoms.

#### References Cited

##### UNITED STATES PATENTS

15 2,653,910 9/1953 Airs et al. ----- 260—327

JAMES A. PATTEN, *Primary Examiner.*

J. D. RANDOLPH, *Assistant Examiner.*